

## UNITED STATES PATENT OFFICE

2,123,153

## PRINTING AND OTHER TEXTILE TREATMENTS

Georges Rivat, Lyon, France, assignor to Celanese Corporation of America, a corporation of Delaware

No Drawing. Application March 28, 1936, Serial No. 71,449. In Great Britain April 4, 1935

11 Claims. (Cl. 8—17)

The present invention relates to improvements in printing and other textile treatments and is more particularly concerned with processes for the fixation of color and other effects upon textile materials.

In U. S. application S. No. 48,283, filed November 5, 1935, of which this application is a continuation-in-part, processes are described whereby the existing dyeing affinities of materials made of or containing natural or regenerated cellulose or cellulose derivatives are modified by incorporating in the materials highly molecular or complex nitrogen-containing organic compounds, more especially nitrogen-containing synthetic resins. The incorporation is effected by interaction on the materials of appropriate reagents one of which contains the requisite nitrogen. As indicated in the said specification, incorporation of the above compounds in natural or regenerated cellulose materials generally confers upon the latter an affinity or increases any existing affinity for the basic and acid colors, and decreases or suppresses entirely their affinity for the direct cotton colors.

I have now found that by forming the said compounds on the material very satisfactory fixation of colors thereon may be effected. For example, the textile materials may be colored with any suitable acid, basic or direct colors, and a synthetic resin thereafter condensed on the material so as to fix the color. By this means the ordinary fixation by steaming may be omitted, and a simple washing or treatment with hydro-sulphite, according to the dyestuff used, suffices to remove excess color.

While the fixation of the color according to the present invention may be uniform over the entire material, the most important application of the present invention consists in local fixation of the color so as to produce pattern effects. The local application of a reagent or reagents suitable for the formation in or on the material of a nitrogen-containing synthetic resin or other complex nitrogenous compound may be by any of the usual printing methods, for example a printing roller, engraved plate, stencil or screen printing, e. g. with a silk screen.

In fixing colors locally according to the present invention, the fabric may, for example, be colored uniformly with a suitable dyestuff, and the agents for making the nitrogen-containing synthetic resin thereafter applied locally, and the fabric subjected to conditions suitable for producing the desired condensation, for example drying for 1-2 hours in a stove at 110° C.-120° C.

A simple washing and clearing with hydrosulphite serves to remove color from the unprinted portions.

If desired, in addition to fixing dyestuffs on the materials effects such as ciré effects may simultaneously be fixed on the materials. The fabric may, for example, be uniformly colored as previously indicated and subsequently printed with a paste containing the condensable reagents, then a ciré finish applied and the fabric subjected to the conditions necessary for condensation of the reagents and finally washed. The ciré finish may be imparted by hot calendering, e. g. by passage between a hot steel roller and a roller of compressed paper, preferably rotating at slightly different speeds, whereby the condensation of the reagents may be wholly or in part simultaneously effected. In the latter case a further heat treatment may be given to complete the condensation. In this way colored local ciré effects may be produced, the washing removing the ciré finish on the unprinted portions.

Colored local ciré effects may also be produced by applying locally a dyestuff in admixture with reagents capable of conversion into nitrogenous resins, applying a ciré finish, e. g. by hot calendering, heating to effect a complete formation of resin from the said reagents, and then washing the material to remove the ciré finish from parts of the material free from resin. By omitting the dyestuff uncolored ciré effects may be produced.

The synthetic resins may be produced on the materials from a wide variety of reagents, one or more of which contain nitrogen. For example, they may be produced by condensation of aldehydic or ketonic bodies, for example formaldehyde, acetaldehyde, benzaldehyde, acetone or the like, with aliphatic or aromatic amines or amides, for example urea, thiourea, guanidine and their derivatives, dicyandiamide, aniline, methyl aniline, diphenylamine, benzyl aniline,  $\beta$ -naphthylamine, para-toluene-sulphonamide or other aromatic sulphonamides or N-alkyl or other derivatives thereof. A further group of materials available is the condensation products of gelatine, casein or other albumenoid compounds with formaldehyde, for example. The invention is not, however, confined to condensation products of aldehydic or ketonic bodies with nitrogen-containing organic compounds, since any other nitrogen-containing resinous or highly complex organic compound is suitable. For example, the condensation product of phenol with methylene diphenyl-diamine may be employed. In most

cases, condensation to produce the above mentioned resinous materials may be most advantageously carried out in the presence of catalysts which may be alkaline, acid or neutral.

5 If desired a partial condensation of the resin-forming reagents may be effected prior to applying them locally to textile materials carrying coloring matters, and the condensation completed on the material. For example, a preliminary condensation to produce, for example, the A type of resinous material which is generally soluble in water, may be carried out prior to local application of the reagents to the fabric or other material. Substances such as monomethylol urea 10 or dimethylol urea may for instance be applied locally to material carrying coloring matter and converted to resins on the material by heating. It is for obvious reasons desirable that the final product produced on the material shall be substantially insoluble in water or in aqueous reagents which are customarily applied to the materials as, for example, in dyeing or scouring operations.

15 The following examples illustrate the invention but are not to be considered as limiting it in any way:—

*Example 1*

20 A fabric is printed or aerographed over the whole of its surface with one or more color compositions as follows:—

|                                                                                                                                                                                     | Grams        |
|-------------------------------------------------------------------------------------------------------------------------------------------------------------------------------------|--------------|
| Acid or direct dischargeable dye                                                                                                                                                    | 10-50        |
| Water and gum                                                                                                                                                                       | 950          |
| 35 After drying at the ordinary temperature, the fabric is over-printed by means of a printing roller with a geometric or floral design with a paste of the following composition:— |              |
| Urea or thiourea                                                                                                                                                                    | gms. 100-150 |
| 40 40% formaldehyde                                                                                                                                                                 | ccs. 300-500 |
| Formic acid                                                                                                                                                                         | ccs. 50      |
| Water and thickener to make up to 1000 gms.                                                                                                                                         |              |

45 The fabric is dried, then stoved at 110° C. and, after condensation, subjected to washing with hot water, then to a clearing with sodium hydrosulphite at 70° C.-80° C. The colors are fixed only in the portions overprinted with synthetic resin.

*Example 2*

50 A fabric of natural or artificial silk is printed with the following:—

|                                                   |              |
|---------------------------------------------------|--------------|
| 55 Urea or thiourea                               | gms. 100     |
| 40% formaldehyde                                  | ccs. 300-500 |
| Formic acid                                       | ccs. 50      |
| Dyestuff                                          | gms. 10-50   |
| Water and thickener so as to make up to 1000 gms. | gms. 300-500 |

60 After drying at the ordinary temperature, the fabric is subjected at a high temperature to an operation giving a ciré finish, and is then stoved for 1-2 hours at 110° C. After stoving, the fabric is washed thoroughly in cold water, the printed portions only retaining the ciré finish.

65 The new process may be applied to various textile materials, for example natural silk, cellulose fibers, e. g. cotton, linen, and regenerated cellulose artificial silk, and artificial silk of cellulose acetate or other cellulose esters or ethers. A particularly valuable feature is that dyestuffs having no substantial affinity for the material may be fixed on the material, e. g. acid dyes on cellulose or cellulose acetate textiles. Very valu-

able effects may be obtained by producing colored ciré effects upon crêpe fabrics, e. g. fabrics constructed with highly twisted regenerated cellulose threads. In this case the crêpe effect is destroyed on the portions on which resin has been fixed, with the result that a pattern of smooth colored areas on a crêpe ground may be obtained. These effects are resistant to washing.

70 Having described my invention what I desire to secure by Letters Patent is:—

1. Process of producing colored ciré effects upon textile materials, which comprises applying a dyestuff to at least parts of the materials, impregnating a portion only of the dyestuff-bearing part of the material with reagents capable of conversion into a nitrogenous resin by the action of heat, imparting a ciré finish to the material by calendering, completing the formation of the said resin from said reagents by heating, and thereafter removing dyestuff and ciré finish from parts of the material free from resin.

2. Process of producing colored ciré effects upon cellulose textile materials, which comprises applying an acid dyestuff to at least parts of the materials, impregnating a portion only of the dyestuff-bearing part of the material with reagents capable of conversion into a nitrogenous resin by the action of heat, imparting a ciré finish to the material by hot calendering, completing the formation of the said resin from said reagents by heating, and thereafter washing the material to remove dyestuff and ciré finish from parts of the material free from resin.

3. Process for the production of colored ciré effects upon textile materials, which comprises applying locally to said materials a dyestuff in admixture with reagents capable of conversion into a nitrogenous resin by the action of heat, imparting a ciré finish to the material by hot calendering, completing the formation of the said resin from said reagents by heating, and thereafter washing the material to remove the ciré finish from parts of the material free from resin.

4. Process for the production of colored ciré effects upon textile materials, which comprises applying a dyestuff to at least parts of the materials, impregnating a portion only of the dyestuff-bearing part of the material with a mixture of urea and formaldehyde, imparting a ciré finish to the material by calendering, heating the material to complete the formation of resin from the urea and formaldehyde, and thereafter removing dyestuff and ciré finish from parts of the material free from resin.

5. Process of producing colored ciré effects upon cellulose textile materials, which comprises applying an acid dyestuff to at least parts of the materials, impregnating a portion only of the dyestuff-bearing part of the material with a mixture of urea and formaldehyde, imparting a ciré finish to the material by hot calendering, heating the material to complete the formation of resin from the urea and formaldehyde, and thereafter washing the material to remove dyestuff and ciré finish from parts of the material free from resin.

6. Process for the production of colored ciré effects upon textile materials, which comprises applying locally to said materials a dyestuff in admixture with urea and formaldehyde, imparting a ciré finish to the material by hot calendering, heating the fabric to complete the formation of resin from the urea and formaldehyde, and thereafter washing the material to remove the

ciré finish from parts of the material free from resin.

7. Process for the production of colored ciré effects upon textile materials, which comprises applying a dyestuff to at least parts of the materials, impregnating a portion only of the dye-stuff-bearing part of the material with a water-soluble urea-formaldehyde condensation product, imparting a ciré finish to the material by 10 calendering, heating the material to complete conversion of the water-insoluble condensation product to a water-insoluble resin, and thereafter removing dyestuff and ciré finish from parts of the material free from resin.

15 8. Process for fixing ciré effects upon textile materials, which comprises forming a nitrogenous resin on the materials to which the ciré effect has been imparted.

9. Process for fixing colored ciré effects upon 20 textile materials, which comprises forming a nitrogenous resin on the materials to which the

ciré effect has been imparted and to which a dyestuff has been applied.

10. Process for the production of colored ciré effects upon textile materials, which comprises applying a dyestuff to at least part of the material, impregnating at least a portion of the dye-stuff-bearing part of the material with reagents capable of conversion into a nitrogenous resin, imparting a ciré effect to at least part of the material, and then effecting formation of said resin 10 from said reagents on the material.

11. Process for the production of colored ciré effects upon textile materials, which comprises applying to at least part of the material a dye-stuff in admixture with reagents capable of conversion into a nitrogenous resin, imparting a ciré effect to at least part of the material, and then effecting formation of said resin from said reagents on the material.

GEORGES RIVAT. 20